

## UNITED STATES PATENT OFFICE

2,363,331

## METHOD OF MAKING MOTOR FUEL

Joseph Hidy James, Pittsburgh, Pa., assignor to  
 Clarence P. Byrnes, Pittsburgh, Pa., as trustee

No Drawing. Application September 14, 1940,  
 Serial No. 356,833

9 Claims. (Cl. 196—50)

In a number of patents such as United States Patent Nos. 1,697,653 of Jan. 1, 1929 (Reissue 18,522), 1,859,587, 1,948,817, 2,010,085, 2,010,086, 2,036,215, 2,054,571; 2,085,221, and 2,085,499, I have described processes for making partial oxidation products from aliphatic and naphthenic hydrocarbons, such as petroleum fractions, shale oil, and oils from the low temperature distillation of coal. In such process, the vaporized or finely divided hydrocarbon is mixed with oxygen or an oxygen containing gas and passed through a reaction zone, preferably in contact with a catalyst, at a temperature below that of continuous self-sustained complete combustion, and preferably below a red heat.

The product when condensed or absorbed and recovered contains partial oxidation products in a range from alcohols to oxygenated organic acids, including aldehydes, ketones, esters, ethers, lactones, etc. Many or all of these bodies are present in different molecular weights.

In this step of oxidation, I prefer to proportion the variable factors so that a large percentage of alcohols is formed as disclosed in my U. S. Patents 1,759,620 and 1,859,587, with relatively less acid; though this is not essential. In the oxidation step some acids are formed and there are some incidental reactions such as cracking, forming of unsaturated hydrocarbons or derivatives, aromatics, and ring body hydrocarbons to some extent, depending upon the ratios of the variable factors in the partial oxidation step.

The present invention is based upon my discoveries relative to formation of aromatics and naphthenes which I can obtain during cracking or thermal decomposition of the product mixture resulting from the oxidation step. These discoveries are that if certain dehydrating catalysts are employed in the cracking step; they act to eliminate the elements of water (OH and H) from remote points in the hydrocarbon chains, resulting in the formation of material or large percentages of ring compounds such as aromatics or naphthenes in the product. This change is especially desirable in making motor fuels and is enhanced by properly adjusting the thermal conditions of catalytic cracking with catalysts of such a group or class. The preferable type of oxide catalysts in such a class is that of inorganic amphoteric oxides. In this type I have found that aluminum oxides are of high value, though oxides of zinc or tin (or of some rare elements such as gallium) may be used. Such amphoteric oxides have the properties of both acidic and basic oxides, since with strong acids they form salts

such as chlorides, nitrates, and sulfates; while with strong bases they form salts in which the aluminum functions as an acid forming with sodium and potassium their aluminates. I have also found that zinc chloride (especially when anhydrous) also functions similarly as a dehydrating catalyst in cracking of my complex oxidation product and similarly calcium chloride and phosphoric acid anhydride.

The desired dehydrating action between remote hydroxyl groups in the hydrocarbon chains to form ring oxygen derivatives is obtained during thermolysis of such oxidation products particularly with higher cracking temperatures, though such catalysts permit the use of lower reacting temperatures than those normally used. Such catalytic thermolysis of oxidation products from mineral oils may be and preferably is carried out under superatmospheric pressures. After cracking, the product is fractionated, as by distilling, and the fraction within the gasoline or motor fuel range is separated from other and heavier fractions. This contains hydrocarbons, some oxygen compounds, unsaturateds, and aromatic and naphthenic bodies.

In carrying out my improved process for making motor fuels of good or high octane rating, I preferably neutralize or saponify and absorb any acids present in the oxidation product, before cracking. However, this is not essential and may be omitted especially where partial oxidation of petroleum fractions in the vapor phase is used and where the vapor exit stream from the oxidation chamber is passed on through the cracking unit or units. Catalytic cracking as herein disclosed may be carried out either in the liquid phase where the vapors from oxidation are condensed, or in the vapor phase or both. In each case sufficient ring or cyclic compounds of the naphthenic or aromatic types may be formed to impart material anti-detonating characteristics to the resulting motor fuels.

I will now give some specific examples:

*Example 1.*—A portion of ordinary commercial cracked gasoline, oxidized by my well known vapor phase catalytic method disclosed in my United States patents before recited herein and containing different oxygen derivatives in the range from alcohols through aldehydes to and including organic acids with similar derivatives of different molecular weights, was subjected to my vapor phase catalytic cracking step as follows:

A smooth steel tube 2 inches in diameter by 14 inches long was mounted in a hot air bath with a thermocouple in a well in the tube center for

giving the vapor temperature. The tube was filled with catalyst balls about the size of grapes or about 1 centimeter in diameter made of 90% by weight of Baker's C. P. aluminum oxide cemented by about 10% by weight of bentonite having the trade name of Volclay. The weight of catalyst was about 230 grams. The oxidized gasoline liquid was fed into one end of the tube at a rate of about 100 c. c. per hour while the catalyst was kept at about 450° C. The recovery of liquid product from such cracking was 91% by volume, having the following analysis:

| Per cent by volume               |      |
|----------------------------------|------|
| Olefines and oxidized bodies     | 31.4 |
| Aromatic hydrocarbons            | 49   |
| Naphthenic hydrocarbons          | 19.6 |
| Saturated aliphatic hydrocarbons | 0    |

*Example 2.*—A run similar to (1) above, was made with anhydrous zinc chloride as the catalyst and a temperature of 325° C. The yield of liquid product was 91% by volume, and its analysis showed:

| Per cent by volume               |      |
|----------------------------------|------|
| Olefines and oxidized bodies     | 32.2 |
| Aromatic hydrocarbons            | 24.8 |
| Naphthenic hydrocarbons          | 23.8 |
| Saturated aliphatic hydrocarbons | 19.2 |

This again shows violent changes in this complex mixture with a different catalyst and with reactions like the above taking place at a relatively low temperature.

In both cases there was a great increase in the percentage of aromatic and naphthenes, due to the peculiar dehydrating effect of the catalyst, carrying such percentage beyond 15% and preferably beyond 20%, and thus giving material anti-detonating characteristics thereto.

The desired reactions to give the result are probably of two kinds: the hydrogen on carbon atom remote from a carbon atom holding a hydroxyl group reacted with the hydroxyl group; and/or a similar reaction occurred between two remote hydroxyl groups. These are illustrated in the following equations:



In either or both cases ring compounds form to a sufficient extent to give the desired anti-knock-  
ing and high octane rating. The non-condensable vapors and gases from both oxidizing and cracking steps may be polymerized into gasoline, the gases from cracking may be recirculated

through the cracking still to give "nucleating" or alkylation as set forth in other of my copending applications, and many other changes may be made without departing from my invention. The catalytic cracking with my improved catalysts may be carried out in the vapor or liquid phase or both. The oxidation may be carried out in the liquid phase, though I prefer my vapor phase process.

10 I claim:

1. In the method of making motor fuel, the steps comprising partially oxidizing a petroleum fraction in the presence of free oxygen to produce a product containing a mixture of oxygen derivatives of hydrocarbons of different molecular weights in the range from aliphatic alcohols to oxygenated organic acids, thereafter thermally decomposing at a temperature of at least about 325° C. a portion of the product containing hydrocarbons of greater carbon content than gasoline under superatmospheric pressure in the presence of a dehydrating catalyst capable of dehydrating the hydrocarbons under said thermal decomposing conditions to produce a fuel of lower average carbon content than said product and which contains cyclic bodies to a material amount, and then fractionating the cracked product to produce motor fuel.

2. In the method of making motor fuel, the steps comprising partially oxidizing a petroleum fraction containing a mixture of normally liquid hydrocarbons of different molecular weight from the group of aliphatic and naphthenic hydrocarbons in the presence of free oxygen to produce a product containing a mixture of oxygen derivatives of hydrocarbons of different molecular weights in the range from aliphatic alcohols to oxygenated organic acids, thereafter thermally decomposing at a temperature of at least about 325° C. a portion of the product containing hydrocarbons of greater carbon content than gasoline in the presence of a dehydrating catalyst capable of dehydrating the hydrocarbons under said thermal decomposing conditions to produce a fuel of lower average carbon content than said product and which contains cyclic bodies to a material amount, and then fractionating the cracked product to produce motor fuel.

3. In the method of making motor fuel, the steps comprising partially oxidizing a petroleum fraction in the vapor phase at an elevated temperature in the presence of free oxygen to produce a product containing a mixture of oxygen derivatives of hydrocarbons of different molecular weights in the range from aliphatic alcohols to oxygenated organic acids, thereafter thermally decomposing at a temperature of at least about 325° C. a portion of the product containing hydrocarbons of greater carbon content than gasoline in the presence of a dehydrating catalyst capable of dehydrating the hydrocarbons under said thermal decomposing conditions to produce a fuel of lower average carbon content than said product and which contains cyclic bodies to a material amount, and then fractionating the cracked product to produce a motor fuel.

4. In the method of making a motor fuel, the steps comprising partially oxidizing a petroleum fraction in the vapor phase at an elevated temperature in the presence of free oxygen to produce a product containing a mixture of oxygen derivatives of hydrocarbons of different molecular weights in the range from aliphatic alcohols to oxygenated organic acids, thereafter thermally decomposing at a temperature of at least about

325° C. a portion of the product containing hydrocarbons of greater carbon content than gasoline in the vapor phase in the presence of a dehydrating catalyst capable of dehydrating the hydrocarbons under said thermal decomposing conditions to produce a fuel of lower average carbon content than said product and which contains cyclic bodies to a material amount, and then fractionating the cracked product to produce motor fuel.

5. In the method of making motor fuel, the steps comprising partially oxidizing a petroleum fraction in the presence of free oxygen to produce a product containing a mixture of oxygen derivatives of hydrocarbons of different molecular weights in the range from aliphatic alcohols to oxygenated organic acids, thereafter thermally decomposing at a temperature of at least about 325° C. a portion of the product containing hydrocarbons of greater carbon content than gasoline under higher pressure in the presence of a dehydrating catalyst capable of dehydrating the hydrocarbons under said thermal decomposing conditions to produce a fuel of lower average carbon content than said product and which contains cyclic bodies to a material amount, and then fractionating the cracked product to produce motor fuel.

6. In the method of making a motor fuel, the steps comprising partially oxidizing a petroleum fraction in the presence of free oxygen to produce a product containing a mixture of oxygen derivatives of hydrocarbons of different molecular weights in the range from aliphatic alcohols to oxygenated organic acids, and thereafter thermally decomposing the product at a temperature of at least about 325° C. in the presence of a dehydrating catalyst consisting of a compound of an amphoteric metal capable of dehydrating the hydrocarbons under said thermal decomposing conditions to produce a fuel of lower average carbon content than said product.

7. In the method of making motor fuel, the steps comprising partially oxidizing a petroleum fraction in the presence of free oxygen to produce a product containing a mixture of oxygen derivatives of hydrocarbons of different molecular weights in the range from aliphatic alcohols to oxygenated organic acids, and thereafter thermally decomposing the product at a temperature of at least about 325° C. in the presence of a dehydrating catalyst from the group consisting of aluminum oxide and zinc chloride capable of dehydrating the hydrocarbons under the said thermal decomposing conditions.
8. In the method of making motor fuel, the steps comprising partially oxidizing a petroleum fraction in the presence of free oxygen to produce a product containing a mixture of oxygen derivatives of hydrocarbons of different molecular weights in the range from aliphatic alcohols to oxygenated organic acids, and thereafter thermally decomposing the product at a temperature of at least about 325° C. in the presence of a dehydrating catalyst capable of eliminating hydroxyl elements of water from remote points in the hydrocarbon chains to form ring compounds.
9. In the method of making motor fuel, the steps comprising partially oxidizing a petroleum fraction in the presence of free oxygen to produce a product containing a mixture of oxygen derivatives of hydrocarbons of different molecular weights in the range from alcohols to oxygenated organic acids, thereafter thermally decomposing at a temperature of at least 325° C. a portion of the product containing hydrocarbons of greater carbon content than gasoline in the presence of a dehydrating catalyst capable of dehydrating the hydrocarbons under said thermal decomposing conditions to produce a motor fuel of lower average carbon content than that of the said partial oxidation product and which contains a material proportion of cyclic bodies.

JOSEPH HIDY JAMES.